

1,339,094.

F. C. BOWMAN.

PREFORMED EXPANSION JOINT STRIP.

APPLICATION FILED FEB. 21, 1914.

Patented May 4, 1920.

2 SHEETS—SHEET 1.

Fig. 1.



Witnesses:

Clarence Perdue

Catherine Doran.

Inventor  
Ford C. Bowman  
By James N. Ramsey  
Attorneys

1,339,094.

F. C. BOWMAN,  
PREFORMED EXPANSION JOINT STRIP.  
APPLICATION FILED FEB. 21, 1914

Patented May 4, 1920.

2 SHEETS—SHEET 2.



Witnesses:

Clarence Perdew  
Catherine Oran

Inventor  
Ford C. Bowman  
By James A. Ramsey  
Attorney

# UNITED STATES PATENT OFFICE.

FORD C. BOWMAN, OF WYOMING, OHIO, ASSIGNOR TO THE PHILIP CAREY MANUFACTURING COMPANY, OF LOCKLAND, OHIO, A CORPORATION OF OHIO.

## PREFORMED EXPANSION-JOINT STRIP.

1,339,094.

Specification of Letters Patent. Patented May 4, 1920.

Application filed February 21, 1914. Serial No. 820,179.

*To all whom it may concern:*

Be it known that I, FORD C. BOWMAN, a citizen of the United States, residing at Wyoming, in the county of Hamilton and State of Ohio, have invented certain new and useful Improvements in Preformed Expansion-Joint Strips, of which the following is a specification.

My invention relates to means for providing for the contraction and expansion of street pavements and the like.

The object of my invention is to provide a ready-made expansion joint strip which is cheap to manufacture and of great efficiency and durability in use, as well as being simple, and convenient to handle and install.

My invention consists in the construction, combination and arrangement of parts and in the completed elastic paving joint as an article of manufacture.

In the drawings:

Figure 1 is a sectional perspective view of a brick-paved street showing my invention installed therein;

Fig. 2 is a sectional perspective view of a cement-paved street with my invention installed in position therein;

Fig. 3 is a perspective view of part of my expansion joint strip; and

Fig. 4 is a similar view of a modification thereof.

While my invention is adapted for various uses, I have illustrated and described it with special reference to street pavements.

The expansion joint strip constructed according to my invention comprises a body of a relatively thick cross-section of asphaltic compound of board like formation and having relatively thin reinforcing and retaining side surfacing sheets of exteriorly non-adhesive fibrous material, such as felt, or any suitable elastic material which is capable of compression and expansion or other similar non-adhesive reinforcing and retaining material. These surfacing sheets are mounted directly upon the surface of the asphaltic body and held thereon by the adhesive and sticking qualities of the asphalt, and when so mounted thereon give to the completed product the quality of non-adhesiveness to adjacent layers when placed upon or against each other in storing or handling the same, thus completely elimi-

nating the danger of the joints sticking together, particularly in warm weather or when in a warm place.

I prefer to construct the joint strip 1 as shown in Fig. 3, with relatively thin layers of wool-felt 2 and 3, saturated with asphaltic cement or compound, upon the sides of the relatively thick body 4 of asphalt, thereby forming a "sandwich" joint of considerable elastic qualities and one which lends itself readily to varying conditions such as irregularities in the abutting side walls of the pavement such as an offset or corner 5, in Fig. 1, around and to which said joint may be readily fitted to completely fill the same, the heavy body of asphalt readily yielding and shifting its mass between the relatively thin layers to conform to such conditions.

The surfacing and reinforcing layers serve to hold the relatively large body of comparatively inexpensive asphaltic material from running or shifting under pressure or otherwise out of its normal predetermined limits between said surfacing material and when constructed as shown in Fig. 3 is considerably reinforced and strengthened so as to withstand undue wearing and abrasive action due to traffic over the paved street under varying conditions of contraction and expansion of the pavement and of the joint. This construction also prevents the joint strip from warping, buckling, cracking or splitting.

In the manufacture of my invention the viscous asphaltic material 4 is formed in a semi-liquid state and is deposited upon one layer 2 of the surfacing material, and by means of rollers spread out to the desired thickness upon said surfacing material 2 and is then passed beneath the other layer 3 of surfacing material and compressed thereagainst; and the combined layers of asphaltic material 4 and surfacing material 2 and 3 are passed between rollers to compress the asphaltic material 4 to the proper density and to thoroughly bring its reinforcing surfacing sides 2 and 3 into adhesive relationship throughout their adjacent surfaces, to form a substantially unitary structure 1 which may be readily and easily handled like a board, but which possesses all of the elastic and non-adhesive properties, and other properties as above pointed out.

After the layers have been thus secured together they are cut into strips of suitable length and width, usually five feet long by six inches in width; the width and thickness varying according to the conditions to be met. I prefer to form the joint 1 of various sizes from  $\frac{1}{2}$  to 1 inch in thickness. It may be readily cut to any desired length just previous to laying it, and its use is very 10 convenient in this respect.

If, for any reason, there should be any cracks or voids 6 in the relatively thick body of asphaltic material 4 the relatively thin layers 2 and 3 of reinforcing surfacing 15 material will support and hold said relatively large body 4 in proper effective position while in storage or transit or in handling, installing or use; so that it forms a sufficiently strong and resisting structure 20 edgewise when placed in position in the street, and at the same time possesses adequate contracting and expanding qualities crosswise of said strip.

My invention is capable of some modification and variation from the structure as above described, as for instance, while I prefer to construct the article in the form of a sandwich joint, the joint strip 1<sup>a</sup> may be formed with a reinforcing and outwardly 30 non-adhesive surface 7 upon one side only of the plastic material 4<sup>a</sup>, as shown in Fig. 4; in which case greater care to prevent the joints 1<sup>a</sup> from sticking together during storage and handling is necessary.

35 My improved ready-made expansion joint strip constitutes a thoroughly practical and reliable substitute for the joints that have heretofore been formed during the process of construction of the pavement, as by temporarily placing strips of wood between the different portions of the paving and then withdrawing the strips and pouring melted material into the space thus left. Coal-tar pitch, asphalt and other bituminous materials have been used to form joints 40 in this manner. Such methods involve the extra labor of inserting and removing the wood strips; and also involve special apparatus and extra labor for melting the material, as well as involving considerable waste of the material in handling, and danger of burning the material in melting, as well as of injury to the workmen. With all this inconvenience and extra expense, 45 the results are not satisfactory or uniform, because there is uncertainty as to the character and quality of a joint thus made by melting and pouring the material. With the practical and reliable ready-made joint 50 which I have invented, the joints may be manufactured complete ready for insertion when the pavement is laid, and may be laid with no more labor than has been required to lay the temporary wood strips. With 55 the joints all made in the same factory by

the same workmen, under uniform conditions not involving distribution of material and apparatus over the field of construction, it is possible to insure a uniform product and allow the nature and quality of the 70 product to be accurately governed or varied to suit the practical conditions met with in different paving projects or to suit the requirements of those having charge of the construction in the different projects.

75 Another disadvantage attending the use of coal-tar pitch, asphalt or other material melted and poured to form the joints, and which is obviated by my invention, is the tendency of the material poured into the space, to form the joint, to run to the lowest part of the joint and leave the higher parts void, under conditions of extremely high temperature, as during hot weather. Thus, in street paving which has considerable 85 crowning, the melted and poured joint will often be found to have become depleted in the high part of the street at the middle, as at A in Fig. 2, and an excess of the material will have collected at the low points at the 90 sides of the street, as at B in Fig. 2. This trouble is also met with in melted and poured joints running longitudinally of the paving, as at C in Figs. 1 and 2, if the paving is longitudinally inclined.

95 My improved ready-made paving joint strip, with the bituminous material of sufficient bulk to give the required thickness to the joint, but with the flanking layers of fibrous material intimately joined therewith and formed, not by melting and pouring the bituminous material, but by pressing it into its intimate relation with the fibrous material, is found in practice to maintain its even distribution of the material throughout 100 the length of the joint, regardless of the difference in elevation between different parts of the structure.

105 To substitute a ready-made paving joint strip constructed entirely of a strip of asphalt or other bituminous material or with the reinforcement inclosed therein, is objectionable, because of the adhesive character of its surface, making storage and handling extremely difficult without damage to 110 such ready-made joints due to their adhering to each other. The flanking fibrous strips or layers, while intimately associated with the bituminous material, present non-adhesive surfaces outward with the bituminous material exposed only on the edges; and there is no trouble experienced in storage or handling, and no damage or waste to the material, because each piece of the ready-made joint strip is self-contained and 115 distinct and remains so, even when stored for a considerable time with the pieces in contact with each other.

120 The modification shown in Fig. 4, where the fibrous material is associated with the 125

body of bituminous material upon only one side of said body, is inferior to my preferred construction with the fibrous material on both sides; but is found to be 5 superior to melted and poured joints and to ready-made joint strips with both sides of the bituminous body exposed. With the fibrous material on one side only of the bituminous body a non-adhesive powdered 10 coating, or a very thin non-adhesive coating of any kind, will prevent sticking of the pieces together in storage; and such a thickness of fibrous material on one side of the bituminous body lends considerable 15 stability to the joint after it is installed, and will generally prevent displacement of the material such as takes place in the other kinds of joints before mentioned.

The exposure of the bituminous material 20 on the edges, while being unobjectionable as above pointed out, also permits considerable economy of construction of the article as compared with ready-made joints where attempt is made to inclose the bituminous 25 material on one or both edges; and the efficiency of the joint for compensating expansion and contraction is also somewhat increased. Thus it is entirely practicable to manufacture my improved paving joint by 30 rolling the bituminous material and its reinforcement together and then cutting it into strips of the desired width and length giving the strips straight parallel edges, which are not produced in merely the rolling 35 operation, but which are thus readily trimmed in the cutting, so that a neat and accurate product is attained. Structures of this character involving reinforcement or covering at the edges are produced by 40 pouring the bituminous material in a melted condition into the reinforcing cover; and these structures therefore differ in properties from the joint which is poured directly into the space in the paving only in that 45 they are portable, as will be more fully pointed out herein.

By making the reinforcing material substantially conterminous with the bituminous material along both of the longer 50 edges of the strip which form the top and bottom when the strip is in position in the paving, the joint is given its highest degree of freedom to change its thickness throughout its extent, because there is an 55 entire absence of reinforcing material transversely of the joint, which while it may be more or less elastic when presented flatwise in the structure, as are the thicknesses of reinforcing material in my improved paving 60 joint, will not manifest their elasticity when pressure is imposed upon them edge-wise as it must be if such material is disposed across the paving joint either at the top or bottom edge or at the ends of the strip.

65 When thus disposed this material will

buckle and produce a disrupting action upon the bituminous interior or otherwise produce a distorting effect upon the joint when the compressing strain is imposed upon it.

70 My improved paving joint strip also has considerably more elasticity than the joint formed entirely of the bituminous material, either by melting or pouring or in a ready-made joint composed only of the bituminous material, or a ready-made joint strip with the reinforcement embedded therein, especially where the embedded reinforcing material is not elastic. With a comparatively thin layer of fibrous material on one 75 or both sides of the bituminous body, yet with considerable thickness to this layer, such as felt or paper affords, this fibrous reinforcement receives the first impact upon expansion of the paving structure, and will 80 yield considerably thereunder, and will very effectively regain its original bulk upon contraction of the paving structure. The necessity of becoming compressed is 85 imposed upon the bituminous body itself 90 only under extreme conditions of expansion, and such elasticity as it naturally possesses will be found sufficient under such conditions and also upon the contraction of the paving structure which follows such extreme conditions.

95 Melted and poured paving joints, especially those formed of coal-tar pitch, are very uncertain in their action under conditions of expansion and contraction of the 100 paving structure, being either too brittle to afford the required elasticity, or, under conditions of high temperature, being greatly softened and pressed out of the joint and left protruding therefrom upon the contraction of the structure, to be worn away and wasted, with the result that the joint is 105 depleted and deteriorated and soon destroyed. This is also true of ready-made joint strips composed entirely of the bituminous material or made with embedded reinforcement, because such material must be of about the same consistency and properties of the melted and poured joint on account of its molded construction and on account of the exposure of the bituminous material without exterior reinforcement. My improved ready-made joint strip, by having the exterior reinforcement, may be made by pressing the different elements of 110 the structure together. This insures a bituminous body of high and practically uniform density, which will not be extruded so objectionably under high temperature, and which will be protected at the surface by 115 the exterior fibrous reinforcement, which will also relieve the bituminous body of the greater part of the required compression under expansion of the paving structure, as 120 before described.

Having fully described my invention, what I claim as new and desire to secure by Letters Patent is:

1. As an article of manufacture, an expansion joint formed of plies of saturated, waterproofed, flexible, elastic material independent of each other, a layer of greater thickness than the said plies of suitable bituminous material bonding said plies in engagement with, but separate from, each other, the whole forming a non-deteriorating, unitary, board-like structure formed by compression.
2. As an article of manufacture, an expansion joint formed of a ply of flexible, elastic material saturated with asphalt, a layer of asphalt of greater thickness than said ply superposed upon said saturated ply and compressed into engagement therewith to form a unitary, board-like structure.
3. As an article of manufacture, an expansion joint formed of plies of saturated

waterproofed flexible elastic material and a layer, having a greater thickness than the said plies, of suitable bituminous material, bonding said plies and spacing them, the whole forming a non-deteriorating unitary board-like structure. 25

4. As an article of manufacture, an expansion joint formed of a ply of flexible elastic material saturated with asphalt and a layer of asphalt of greater thickness than said ply superposed upon and in engagement therewith forming a unitary board-like structure. 30

5. As an article of manufacture, an expansion joint formed of a ply of flexible elastic material and a layer of asphalt of greater thickness than said ply superposed upon and in engagement therewith. 35

FORD C. BOWMAN.

Witnesses:

H. C. INNES,  
JAMES N. RAMSEY.